

## UNITED STATES PATENT OFFICE

2,603,582

PRODUCTION OF LAUNDERABLE SEMISTIFF  
FABRICS OR ARTICLES OF WEARING AP-  
PAREL

Eric Higgins, Punchetts, Tewin Wood, England

No Drawing. Application June 12, 1945, Serial  
No. 599,128. In Great Britain May 23, 1944Section 1, Public Law 690, August 8, 1946  
Patent expires May 23, 1964

6 Claims. (Cl. 154—115)

1

This invention relates to the production of launderable semi-stiff fabrics and articles of wearing apparel and is concerned with fabric articles involving in their production the amalgamation of plies of fabric, one at least of which—which may for convenience be called the operative ply—contains strands or elements of cellulose acetate, and strands or elements of cotton.

It is well known in the art to effect the amalgamation of the plies or laminations by first treating them—or at least the operative ply—with a solvent for the cellulose acetate and then subjecting the superimposed plies or laminations to pressure accompanied by heat. One such process which has proved successful in practice is disclosed in the specification of British Letters Patent No. 419,208.

This process, however, involves the use of solvents which is open to certain obvious objections. It has, therefore, been suggested, from time to time, to eliminate the use of solvents by plasticising the operative ply consisting of or containing the cellulose acetate and many plasticisers are known in the art and it has already been suggested to use for the purpose an aqueous dispersion of a plasticiser, such dispersion containing an organic derivative of cellulose.

Hitherto, it has been thought that it was desirable to induce as much as possible of the plasticiser to be absorbed by the organic cellulose acetate constituent of the fabric and the only instance known of where the use of an emulsion in the form of an aqueous dispersion of the plasticiser was suggested, for the purpose of rendering the plasticised fabric less greasy to the touch, the dispersion employed essentially contained an organic derivative of cellulose. The result of this must inevitably be that, while the cellulose acetate constituent of the fabric could be made to absorb any desired amount of plasticiser, dependent on the period of immersion, the cotton constituent of the fabric, would not take up the plasticiser, except, maybe, to a negligible extent in the form of a thin skin.

The object of the present invention is to provide a process by which any desired ratio of plasticiser content as between the cellulose acetate constituent of the fabric and the cotton constituent can be attained. This object can be accomplished by the use of an aqueous emulsion of the plasticizer of predetermined concentration.

The present invention is based upon the conception, in contradistinction to the earlier proposal, that the cotton constituent of the com-

2

posite fabric should be induced to take up a controlled amount of the plasticiser and the object of the present invention, therefore, is to provide a process by means of which a fabric can be produced in which there is a controlled differential ratio between the amount or quantity of plasticiser contained in the cellulose acetate constituent of the fabric and the cotton constituent of the fabric.

10 The amount of plasticiser in the cellulose acetate is determined as heretofore by the time period during which the fabric is treated with the emulsion and the amount contained in the cotton constituent is controlled, primarily, by the concentration of the emulsion and, secondarily—but quite importantly in the practical carrying out of the process—by the extent to which excess liquid is expressed from the fabric after treatment with the emulsion.

15 It will be understood that the ratio which will give the best results should be ascertained by trial with each particular composite fabric, since the optimum ratio is dependent upon a variety of conditions such, for example, as the structure of the operative ply itself, and, also to a lesser extent, the characteristics of the plies with which it is subsequently to be called upon to bond.

20 From the foregoing it will be seen that the present invention consists of a process for plasticising composite fabric consisting of threads or strands of both cellulose acetate and threads or strands of cotton, by means of an aqueous emulsion of a plasticiser according to which the composite fabric is immersed in an emulsion of predetermined concentration for a period of time depending on the quantity of plasticiser required to be taken up by the cellulose acetate constituent, whereby the amount of plasticiser retained by the cellulose acetate constituent of the fabric and the amount of plasticiser retained by the cotton constituent of the fabric are selectively controlled, the content of the cellulose acetate constituent being dependent on the period of immersion in the emulsion, and that retained by the cotton constituent being determined by the concentration of the emulsion.

25 More specifically, the invention consists of a process for plasticising composite fabric consisting of threads or strands of both cellulose acetate and threads or strands of cotton, by means of an aqueous emulsion of a plasticiser according to which the composite fabric is immersed in an aqueous emulsion of predetermined concentration for a period of time depending on the quantity of plasticiser required to be taken up by

the cellulose acetate constituent, the fabric being then subjected to a mangling or other expression process for the removal of excess liquid and the fabric is finally dried, whereby the amount of plasticiser retained by cellulose acetate constituent of the fabric and the amount of plasticiser retained by the cotton constituent of the fabric are selectively controlled, the content of the cellulose acetate constituent being dependent on the period of immersion in the emulsion, and that retained by the cotton being determined by the concentration of the emulsion and the degree to which excess liquid is expressed from the fabric prior to final drying.

The invention further includes a plasticised fabric composed of cellulose acetate and cotton having a predetermined plasticiser content in the cellulose acetate constituent and a predetermined plasticiser content in the cotton constituent.

In carrying my invention into practice the operative fabric is manufactured containing the necessary amount and distribution of cellulose acetate threads or elements according to the present practised art, and this fabric is then according to my invention treated with an aqueous emulsion of a suitable plasticiser under conditions in which the plasticiser is selectively substantive to the cellulose acetate so that the distribution of the plasticiser between the operative (cellulose acetate) and non-operative elements of the composite is under control; thereafter the fabric is dried and can be employed precisely as was formerly customary in the art, with the exception that it is not necessary to employ solvents, ultimate "fusion" being brought about merely by the application of heat and pressure.

The operative fabric aqueously plasticised according to my invention may be marketed as such, being a fabric possessing agreeable handling and textile characteristics as susceptible of use in accordance with normal manufacturing procedure as are the operative fabrics now used in the art.

I have found that in order for the operative fabrics to have the desired properties and retain them even after considerable lapse of time, not only must the acetate cellulose contain and retain a sufficient quantity of plasticiser to reduce its melting or softening point to practically realisable and convenient limits, but the non-operative fibres with which it is associated must also contain and retain a proportionate amount of the plasticising agent in order to permit of spreading instead of balling up of the cellulose acetate solid solution when it is subsequently brought to fusion.

This proportionate absorption and fixation of the plasticiser (which would be excessively difficult, if not impossible, to control if working in a non-aqueous medium, and, in the absence of a diluent, would result in excessive proportions of plasticiser in the non-operative threads) is easily controlled when absorption of the plasticiser is effected from a suitable emulsion of the plasticiser in water. That is to say, regulation as regards the non-operative non-substantive fibres is conditioned by the concentration of plasticiser in the emulsion and in the operative substantive element by the duration of the treatment.

A great number of plasticisers are known and used by those skilled in the art and many of these are suitable for use according to my invention. Choice should, however, be guided by the selection of such as are chemically stable, alone and in the presence of water at medium temperatures, say between 60° F. and 200° F., and which

are neutral, slightly soluble in water, and of low volatility per se and in steam at temperatures up to 300° F. On the other hand, it is not necessarily disadvantageous and it may even be desirable for the solvent used to be broken down into water-soluble constituents (uninjurious of course to the ordinary textiles) when subjected to laundry conditions—that is to say to the action of mildly alkaline water at temperatures of 212° F. or thereabouts—since the ultimate removal of the plasticiser increases the strength of the bond in the finished article and its ready removal by ordinary laundering processes is an added advantage. Clearly, cheapness, availability, freedom from strong odour and in a smaller measure freedom from pronounced colour are of general and obvious advantage.

In the preparation of the aqueous emulsions an emulsifying agent will generally be necessary for commercial convenience, and a large number of agents are known and available to those engaged in the art. Choice again should be guided in favour of such agents as are operative in neutral or nearly neutral solutions and are free from action upon the textiles themselves and upon colouring matters employed to decorate them. Free removal from the fabric by laundry processes is clearly a desideratum in such emulsifying agents and clearly it is advantageous if on drying upon the fabric they assist in the retention (by the formation of a film for example) of the non-substantively held plasticiser in the non-acetylcellulosic portion of the composite fabric and hinder its flow or migration. Solely by way of example of a suitable emulsion, and without, be it understood, limiting myself to this particular selection I give a composition of matter which has been found to give the effect claimed in this application in a peculiarly advantageous manner.

500 lbs. of a mixture consisting of 55 per cent by weight of formanilide and 45 per cent of o-formyltoluicide is introduced with intensive stirring into a solution of 24 lbs. of casein in 470 lbs. of water and 12 lbs. of hydrated borax at a temperature of 200° F. or thereabouts. The mixture is passed, whilst being well mixed, once or twice through an homogeniser and the resultant emulsion cooled as quickly as possible. The cold emulsion is stable, contains approximately 50 per cent of its weight of the plasticising mixture and has a pH of about 7.5.

Into such an emulsion the fabric containing the cellulose acetate threads or elements is passed and allowed to remain in the emulsion until the desired amount of plasticiser has been absorbed by the acetate threads, the amount retained by the non-acetate portion of the composite being determined by the concentration of the emulsion and the degree to which the excess fluid is expressed from it before drying.

Thus, if the emulsion be used at a concentration of  $x$  per cent of plasticiser and the goods at the completion of the impregnation be mangled or hydroextracted to an expression of  $y$  per cent, the non-acetate threads on drying will contain

$$y \times \frac{x}{100}$$

per cent of plasticiser no matter how long immersion is contained provided uniform penetration is achieved. On the other hand, the amount of plasticiser absorbed by the acetate constituent will at any chosen concentration of the emulsion be a function of the time of immersion and be but little affected ultimately by the original

concentration of the emulsion or the "expression" left before drying, though clearly the more dilute the emulsion the longer the period of immersion which will be necessary to achieve a given concentration of plasticiser in the acetate elements. In general, elevated temperature will, other things being equal, decrease the time necessary for a given percentage absorption by the acetate.

Thus, separate portions of a composite fabric of all cotton warps and alternated 4 cotton and 2 acetate wefts were passed through the emulsion given as an example and allowed to remain on the batch, a convenient commercial expedient, for varying periods; thereafter they were mangled to 100 per cent expression and dried at 130-140° F. They gave the following figures:

Left on the batch 5 minutes 50 per cent plasticiser in cotton, 50 per cent plasticiser in acetate.

Left on the batch 10 minutes 50 per cent plasticiser in cotton, 75 per cent plasticiser in acetate.

Left on the batch 20 minutes 50 per cent plasticiser in cotton, 117 per cent plasticiser in acetate.

The three dried fabrics were then separately used as an interlayer between two pieces of cotton poplin and were ironed for 30 seconds from back and front with a tailor's iron at 200° F. The adhesions measured on a 1" strip were respectively 90, 170, and 190 grammes and, after laundering, 700, 950 and 1,150 grammes. However, when portions of the sample containing 50 per cent of plasticiser in cotton and acetate were ironed for a period of 2 minutes at the same temperature, or for the same time (30 seconds) with an iron at 240° F. their adhesion rose to 170 grammes and, after laundering, to 1,050 grammes.

The degree of plasticisation to be achieved depends upon the precise requirements of the user. Clearly, the lower the temperature and/or the greater the speed at which it is desired to combine and/or stiffen the fabrics, the higher the proportion of plasticiser necessary in the cellulose acetate and in general the greater the difference in the primary and laundered strength of adhesion. For any particular conditions of temperature-pressure and speed of fusion there will be a corresponding optimum plasticiser concentration below which the laundered strength will be less than that realisable with the acetate cellulose present but above which for a considerable range of increased concentration there will be no considerable increase in ultimate adhesion. If the proportion of plasticiser introduced into the cellulose acetate is permitted to reach high figures (for example 300 per cent or more) the fusion or solution temperature of the plasticised threads may fall so low that extreme care in heat regulation and/or time of treatment would be necessary to prevent such an excessive flow of the mass as to reduce the primary adhesion strength below practicable limits and/or spread the adhesive into a continuous and impermeable layer; moreover, the operative fabric would tend to become sticky and clammy in handling and cease to be a merchantable article, at least in markets in which fabrics normally find application.

Nevertheless, where such operative fabrics are to be employed when manufactured for imme-

diate incorporation in semi-stiffened tissue (for example as a continuous process within one factory) such extreme plasticisation may be employed with advantage, adhesion being then accomplished by heavy pressure (for example by a calender) at ordinary air—or but slightly elevated temperatures, the tissue passing at once to a laundering treatment. The mutual adjustment between the cost of the plasticiser and the advantage of low-temperature and/or high-speed working cannot be laid down since it is dependent upon variable conditions extraneous to the process.

It is clear that, instead of padding and beaming, the differential absorption can be timed in a variety of ways well known in the art; for example, the operation can be conveniently carried out on a jig or dyeing machine, the time factor being controlled in accordance with the length of the pieces and the number of "ends" given. Thus a fabric (as described before), treated on the jig with the emulsion already given, gave the following figures:

| 25 | Treatment             | Time of Immersion     | Adhesion         |
|----|-----------------------|-----------------------|------------------|
|    |                       |                       | after laundering |
| 30 | Straight through..... | about 1 minute.....   | grammes 890      |
|    | One end.....          | about 5 minutes.....  | 950              |
|    | Two ends.....         | about 10 minutes..... | 1,350            |
|    | Four ends.....        | about 20 minutes..... | 1,350            |

It will be seen from the foregoing that I have by my invention provided a process possessing manifest advantages. The elimination of the use of volatile solvents of which relatively large volumes are required—much of which is necessarily wasted—results in economy. Such solvents are usually highly inflammable with the consequent risks of fire, demanding special equipment and moreover, where solvents are used, the operation is of a type to which the trades involved are not accustomed. With the use of my special plasticised operative ply nothing more than an ordinary ironing operation either by means of a hand iron a laundry press or other equipment with which operatives are familiar suffices to ensure a satisfactory product.

The use of the aqueous emulsion permits adequate control of the degree of plasticising of the material both as a whole and also the ratio of distribution of the plasticiser as between the acetyl-cellulosic and non-acetyl-cellulosic constituents of the material.

Thus the operative ply material can readily be produced to meet varying requirements by changes in the concentration of the aqueous emulsion and the immersion time period.

I claim:

1. A plasticiser for cellulose acetate adapted to be used in the production of launderable semi-stiff fabrics from laminations at least one of which laminations consists of both cellulose acetate and cotton, which plasticiser consists of an aqueous emulsion of the following constituents, in approximately the following proportions in parts by weight:

|                       | Parts |
|-----------------------|-------|
| 70 Formanilide .....  | 275   |
| o-Formyltoluide ..... | 225   |
| Casein .....          | 24    |
| Hydrated borax .....  | 12    |
| Water .....           | 470   |

2. A plasticiser for cellulose acetate adapted

to be used in the production of launderable semi-stiff fabrics from laminations, at least one of which laminations consists of both cellulose acetate and cotton, which plasticiser consists of an aqueous emulsion composed of a mixture of formanilide, o-formyltoluicide having the constitution:



casein, hydrated borax, and water, the said emulsion being prepared by intermixing a mixture consisting of approximately 55 percent by weight of formanilide and approximately 45 percent of o-formyltoluicide and a solution consisting of approximately 24 parts by weight of casein and approximately 12 parts by weight of hydrated borax in approximately 470 parts by weight of water, the mixture and solution being intermixed in the ratio of approximately 500 parts by weight of the mixture to the 470 parts by weight of water.

3. A process for plasticising laminating fabrics consisting of strands of both cellulose acetate and cotton, which comprises preparing a plasticiser composition by intermixing a mixture consisting of approximately 55 percent by weight of formanilide and approximately 45 percent of o-formyltoluicide and a solution consisting of approximately 24 parts by weight of casein and approximately 12 parts by weight of hydrated borax, in approximately 470 parts by weight of water maintained at a temperature of approximately 200° F., the formanilide-o-formyltoluicide mixture being intermixed with the said solution in the ratio of approximately 500 parts by weight of the mixture to the 470 parts by weight of water, cooling the resulting emulsion, and immersing the fabric in the resulting emulsion.

4. A process for producing laminating fabrics composed of strands of both cellulose acetate and cotton, which comprises preparing a plasticiser emulsion by adding a mixture consisting of approximately 55 percent by weight of formanilide and approximately 45 percent of o-formyltoluicide to a solution consisting of approximately 24 parts by weight of casein and approximately 12 parts by weight of hydrated borax in approximately 470 parts by weight of water maintained at a temperature of approximately 200° F., the said mixture being added to the said solution in the ratio of approximately 500 parts by weight of the mixture to the 470 parts by weight of water, rapidly cooling the resulting emulsion, immersing the fabric in the emulsion until the plasticizer is absorbed both by the bottom and by the cellulose acetate, removing the fabric from the emulsion, pressing out excess emulsion from the fabric, and drying the fabric.

5. A process for producing composite laminated fabrics, one layer of the laminated fabrics being an operative layer of fabric consisting of strands of both cellulose acetate and cotton, which comprises preparing a plasticizer emulsion by adding a mixture consisting of approximately 55 percent by weight of formanilide and approximately 45 percent of o-formyltoluicide to a solution consisting of approximately 24 parts by weight of casein and approximately 12 parts by weight of hydrated borax in approximately 470 parts by weight of water maintained at approximately 200° F., the formanilide-o-formyltoluicide mixture being added to the said solution in the ratio of approximately 500 parts by weight of the mixture to the 470 parts by weight of water, cooling the resulting emulsion, immersing the fabric in the emulsion until the plasticizer is absorbed both by the cotton and by the cellulose acetate, removing the fabric from the emulsion, pressing out any excess emulsion from the fabric, drying the resulting operative fabric, placing the resulting operative fabric in juxtaposition with a non-operative fabric, and bonding together the juxtaposed operative and non-operative fabrics by applying heat and pressure until bonding thereof is effected.
6. A plasticized operative fabric for producing a laminated fabric structure, which operative fabric is composed of a cellulose acetate constituent and a cotton constituent, each of the said constituents containing a plasticizer for the cellulose acetate produced by intermixing a mixture consisting of approximately 55 percent by weight of formanilide and approximately 45 percent of o-formyltoluicide and a solution consisting of approximately 24 parts by weight of casein and approximately 12 parts by weight of hydrated borax in approximately 470 parts by weight of water, the mixture and solution being intermixed in the ratio of approximately 500 parts by weight of the mixture to the 470 parts by weight of water.

ERIC HIGGINS.

## REFERENCES CITED

The following references are of record in the file of this patent:

## UNITED STATES PATENTS

| Number    | Name           | Date          |
|-----------|----------------|---------------|
| 1,962,763 | Christopher    | June 12, 1934 |
| 1,971,522 | Dunham         | Aug. 28, 1934 |
| 2,101,574 | Dangelmajer    | Dec. 7, 1937  |
| 2,165,506 | Platt et al.   | July 11, 1939 |
| 2,228,158 | Teale          | Jan. 7, 1941  |
| 2,316,146 | Adams          | Apr. 13, 1943 |
| 2,326,128 | Dreyfus et al. | Aug. 10, 1943 |
| 2,326,190 | Whitehead      | Aug. 10, 1943 |
| 2,334,607 | Christopher    | Nov. 16, 1943 |
| 2,351,109 | Corwin         | June 13, 1944 |
| 2,409,703 | Lyem           | Oct. 22, 1946 |
| 2,409,704 | Lyem           | Oct. 22, 1946 |